



US007445648B2

(12) **United States Patent**  
**Hudson et al.**

(10) **Patent No.:** **US 7,445,648 B2**  
(45) **Date of Patent:** **Nov. 4, 2008**

(54) **WAX BLENDS FOR CANDLES WITH IMPROVED PROPERTIES**

(75) Inventors: **Carl Wayne Hudson**, Woolwich Township, NJ (US); **Christopher Jeffrey Kent**, Paulsboro, NJ (US); **Anthony Patrick Hennessy**, Epsom (GB)

(73) Assignee: **ExxonMobil Research and Engineering Company**, Annandale, NJ (US)

(\*) Notice: Subject to any disclaimer, the term of this patent is extended or adjusted under 35 U.S.C. 154(b) by 670 days.

(21) Appl. No.: **10/943,736**

(22) Filed: **Sep. 17, 2004**

(65) **Prior Publication Data**

US 2005/0086853 A1 Apr. 28, 2005

**Related U.S. Application Data**

(60) Provisional application No. 60/513,866, filed on Oct. 23, 2003.

(51) **Int. Cl.**

**C10L 5/00** (2006.01)

(52) **U.S. Cl.** ..... **44/275**; 206/21

(58) **Field of Classification Search** ..... **44/275**; **208/21**

See application file for complete search history.

(56)

**References Cited**

U.S. PATENT DOCUMENTS

|                 |   |         |                         |          |
|-----------------|---|---------|-------------------------|----------|
| 3,046,101 A     | * | 7/1962  | Tench .....             | 44/275   |
| 3,069,346 A     | * | 12/1962 | Tench .....             | 208/21   |
| 3,356,469 A     |   | 12/1967 | Stephenson et al. ..... | 44/6     |
| 4,224,204 A     |   | 9/1980  | Nichols et al. .....    | 260/23 H |
| 4,855,098 A     |   | 8/1989  | Taylor .....            | 264/103  |
| 6,534,573 B1    |   | 3/2003  | Mace et al. .....       | 524/277  |
| 2002/0040863 A1 |   | 4/2002  | Cody et al. .....       | 208/18   |
| 2003/0101640 A1 |   | 6/2003  | Wood et al. .....       | 44/275   |

\* cited by examiner

*Primary Examiner*—Cephia D Toomer

(74) *Attorney, Agent, or Firm*—Estelle C. Bakun

(57) **ABSTRACT**

The present invention relates to a set of wax parameter specifications that will produce candles with improved properties. Specifically, the present invention relates to a blend of waxes that produces container candles with surprising properties and eliminates or minimizes the use of costly microwax, polymers or additives. More specifically, this invention relates to a blend for and method of producing container candles that demonstrates the improved properties of low shrinkage, little oil bleed, enhanced opaqueness and creamy appearance and enhanced fragrance retention.

**11 Claims, 6 Drawing Sheets**



FIGURE 1



FIGURE 2



FIGURE 3



FIGURE 4



FIGURE 5

iso-Paraffin Content of Typical Microwax:



FIGURE 6

iso-Paraffin Content of Preferred Wax of this Invention (LS 1360), HM FRW & Microwax:



## WAX BLENDS FOR CANDLES WITH IMPROVED PROPERTIES

This application claims the benefit of U.S. Ser. No. 60/513,866 filed Oct. 23, 2003.

### FIELD OF INVENTION

The present invention relates to a set of wax parameter specifications that will produce candles with improved properties. Specifically, the present invention relates to a blend of waxes that produces container candles with surprising properties and eliminates or minimizes the use of costly additives. More specifically, this invention relates to a blend for and method of producing container candles that demonstrates the improved properties of low shrinkage, little oil bleed, enhanced opaqueness and creamy appearance and enhanced fragrance retention.

### BACKGROUND OF INVENTION

Although candles have been produced for millennia, certain problems in candle production still remain. Specifically, candle producers desire candle waxes that demonstrate little or no shrinkage, little or no oil bleed, a pleasing and stable appearance and the ability to retain fragrance. Candles are traditionally made of petroleum derived waxes with mostly normal paraffin (n-paraffin) content, lower molecular weights, and therefore lower melting points. While candles with high n-paraffin content retain the proper color and texture desired by candle makers, they are often plagued by excessive shrinkage and poor fragrance retention.

While all of the above properties are important to candle makers, the most important property is the melting point of the wax. Candle makers use Fully Refined Waxes ("FRW"), which usually have less than 1% oil content, as the largest, if not only, wax type in their candles. On occasion, candle makers add microwax or polymers, to enhance the candle's properties, but these additives are costly relative to the wax. Low Melting ("LM") point wax usually melts at 128° F. (53° C.) or less. Waxes of this type are typically used for container candles, i.e., religious novena candles and decorative, fragranced jar candles. Typically LM FRW is gray in appearance and demonstrate relatively high shrinkage. Mid Melting ("MM") point waxes usually melt between 128 and 145° F. (53-63° C.) and are often used for higher quality container candles and free standing candles. MM RHC™ FRW are gray in appearance and demonstrate only slightly less shrinkage than LM FRW.

High Melting ("HM") point waxes, melting at greater than 145° F. (63° C.), are not commonly used in the candle industry. While waxes of this type typically demonstrate less shrinkage than either LM or MM RHC™ waxes, other significant disadvantages have prevented their use in the candle industry. HM FRW waxes are not used as candles because they exhibit a "tunneling" effect. That is, the candle burns straight down into the candle, leaving walled sides. The tunneling effect has proven highly commercially unattractive for both jar and stand-alone candles. The tunneling effect is caused because the "pool" of liquid wax that forms on the top surface of a burning candle does not extend far from the flame, due to the high melting point of the wax. Thus, the candle tends to be consumed unevenly, carving out a cylinder in the center of the candle. A solution to this problem would be to use a larger wick, but this produces a larger and higher flame—again a commercially unattractive option.

Shrinkage is a common problem experienced in candle manufacture. As a molten candle wax solidifies, the volume shrinks. In some cases this shrinkage can be beneficial, for example in helping a poured candle pull away from the sides of a mold making it easier to remove. However, wax shrinkage usually produces an unwanted concave effect on the top of the candle. Candle manufacturers must often re-melt the top portion of the candle or even resort to a second pouring of the candle wax formulation to level the top should excess shrinkage occur. In container candles, shrinkage can lead to candle separation from the side of the container—another undesired effect. Shrinkage has been directly linked to the amount of n-paraffin in the candle wax. Candle waxes containing about 100% n-paraffin will shrink approximately 12 to 15% by volume on cooling. Candle waxes containing about 75% n-paraffin will shrink approximately 8 to 12% by volume on cooling. Candle waxes containing about 50% n-paraffin will shrink approximately 6 to 8% by volume on cooling.

Several methods have been developed in an effort to control excessive shrinkage in container candles. Typically shrinkage is controlled by introducing components that will disrupt the n-paraffin crystal formation. Historically, the addition of high molecular weight isoparaffins (in the form of microwax or petrolatum), oxygenated molecules (such as 25 carboxylic acids, carboxylate esters) and polyol structures have helped control shrinkage. However, these solutions are usually costly, can alter the color and texture of the candle, and, in some cases, raise the melting point to an unacceptably high level.

Another significant concern for candle makers is oil bleed. Oil bleed can be defined as the migration of oil or oil-type molecules out of and onto the surface of the solid wax. The appearance of oil on the wax candle surface is generally regarded as an unacceptable appearance phenomenon. The oil can be derived from the natural oil content of the petroleum wax or from added oily components in the candle formulation, including fragrance oils and carrier solvents for fragrance packages. Petroleum waxes of all types contain some amount of oil. Fully refined waxes have typically less than 1%, more often less than 0.5%, oil content (as measured by the ASTM D-721 test method). Scale waxes are low oil content slack waxes. With further refinement to improve color and odor, typically by hydrotreatment, scale waxes can be upgraded to semi-refined waxes that can have from 1% to 45 about 5% oil content (as measured by the ASTM D-721 test method). Semi-refined waxes have found limited use in container candles, in spite of their typically lower cost, because of a greater tendency to exhibit oil bleed in a formulated candle.

Historically, methods for improving oil bleed or fragrance 50 hold in candle manufacture include:

1. addition of high molecular weight microwax (derived from bright stock),
2. addition of petrolatum (petroleum jelly),
3. addition of other additives, and
4. rigorous control of process conditions, such as cooling 55 rates and sequences.

While helping to minimize oil bleed, the addition of microwax and modified waxes often causes additional problems of shrinkage (see above). The addition of petrolatum or petroleum jelly is relatively expensive and significantly softens the candle. Other additives can also be expensive and/or can negatively alter the appearance and shrinkage characteristics of the wax and candle formulation. Finally, varying the cooling rates and sequences is labor intensive and often varies 60 with the slightest difference in the underlying candle wax.

Another important attribute for candle manufacturers is the color and uniformity of the raw candle. The impact of raw 65

wax color and appearance on the final candle formulation can be significant. For example, a translucent gray LM fully refined wax will provide a different appearance in a given candle formulation than higher melting, more isoparaffinic wax that has a more cloudy, white-gray appearance. Candle makers typically formulate for a given type of base wax and strive to maintain a consistent color and appearance for each candle formulation. A wax that exhibits a rich, creamy opaque whiteness can provide the candle maker with new and improved options for candle formulation.

#### DESCRIPTION OF THE FIGURES

FIG. 1 is a graphical representation of the Carbon number versus the iso-paraffinic weight percentage at that carbon number for a typical low melting point fully refined wax with a melting point of 126° F.

FIG. 2 is a graphical representation of the Carbon number versus the iso-paraffinic weight percentage at that carbon number for a typical high melting point fully refined wax with a melting point of 156° F.

FIG. 3 is a drawing of the jar used for the shrinkage experiments.

FIG. 4 is a graphical representation of the Carbon number versus the iso-paraffinic weight percentage at that carbon number for a low melting point fully refined wax (MP 126° F.), a high melting point fully refined wax (MP 156° F.), a mid melting point RHCTM wax (MP 135° F.) and a 90:10 blend of the high melting point fully refined wax and the mid melting point RHCTM wax (MP 136° F.) ("LS 1360").

FIG. 5 is a graphical representation of the Carbon number versus the iso-paraffinic weight percentage at that carbon number for a typical microwax.

FIG. 6 is a graphical representation of the carbon number versus the iso-paraffinic weight percentage at that carbon number for the 90:10 blend ("LS 1360"), the High Melting Fully Refined Wax (MP 156) and a typical microwax.

#### SUMMARY OF INVENTION

The present invention comprises a method to produce candles of low shrinkage, low oil bleed, good color and texture and expected superior fragrance retention (due to the low bleed) comprising blending a wax composition such that isoparaffinic content of the original paraffinic wax is increased for carbon numbers between 35 and 60, but not increased by more than about 0.1 wt % for carbon numbers greater than 60 at a given carbon number, and the products produced by this method.

Preferably, the present invention is a wax blend comprising blending a wax composition such that isoparaffinic content of the original paraffinic wax is increased for carbon numbers between 36 and 57, but not increased by more than about 0.1 wt % for carbon numbers greater than 57 at a given carbon number, and the products produced by this method. More preferably, the present invention is a wax blend comprising blending a wax composition such that isoparaffinic content of the original paraffinic wax is increased for carbon numbers between 37 and 55, but not increased by more than about 0.1 wt % for carbon numbers greater than 55 at a given carbon number, and the products produced by this method. Even more preferably, the present invention is a wax blend comprising blending a wax composition such that isoparaffinic content of the original paraffinic wax is increased for carbon numbers between 37 and 50, but not increased by more than about 0.1 wt % for carbon numbers greater than 50 at a given carbon number, and the products produced by this method.

In another embodiment, the present invention comprises a product that exhibits low shrinkage, low oil bleed, good color and texture and superior fragrance retention comprising:

- a) about 75-95 wt % of a first wax having
  - 1. a melting point of between about 128° F. to about 145° F.;
  - 2. an oil content of between about 1 wt % to about 10 wt %;
  - 3. a total paraffins average carbon number of between about 29-33;
  - 4. an iso-paraffin average carbon number of between about 30-34;
  - 5. about 43-57 wt % n-paraffins;
  - 6. a 95% carbon # spread of 12-16;
  - 7. with the wt % of C24 or less being less than about 10%;
  - 8. with the wt % of C34 or greater being less than about 30%;
  - 9. with the wt % of C38 or greater being less than about 10%; and
- b) the remainder being a second wax having
  - 1. a melting point greater than about 152° F.;
  - 2. an oil content of less than about 1 wt %;
  - 3. a total paraffins average carbon number of between about 36-40;
  - 4. an iso-paraffin average carbon number of between about 38-42;
  - 5. about 43-57 wt % n-paraffins;
  - 6. a 95% carbon # spread of 19-25;
  - 7. with the wt % of C24 or less being less than about 5%;
  - 8. with the wt % of C34 or greater being greater than about 60%; and
  - 9. with the wt % of C38 or greater being greater than about 40%.

A preferred form of this embodiment would be a wax blend wherein the first wax was provided as about 80 to 92.5 wt % of the total blend. A more preferred form of this embodiment would be a wax blend wherein the first wax was provided as about 85 to 90 wt % of the total blend. An alternate embodiment comprises any of the embodiments that varied the amount of the first wax in the wax blend where the melting point of the first wax was preferably about 129° F. to about 140° F., and more preferably the melting point of the first wax was preferably about 131° F. to about 139° F. Another alternate embodiment encompasses any of the changes to the amount of the first wax in the final blend or the properties of the first wax listed above and preferably modifying the oil content of the first wax to be between about 1 wt % to about 7 wt %, more preferably between about 1 wt % and about 5 wt %. Another alternate embodiment of this embodiment encompasses any of the modifications to the first wax noted above and modifying the melting point of the second wax such that it is preferably greater than about 154° F., more preferably greater than about 156° F. Another alternate embodiment of this embodiment encompasses any of the modifications noted above to either the first or second wax and further modifying the second wax such that it preferably has an oil content of less than about 0.75 wt %, more preferably less than about 0.5 wt %.

As used in this specification, the oil content of a wax is determined using test method ASTM D-721. As used within this specification the total amounts of paraffins and iso-paraffins at a carbon number is determined by the ASTM D-5442 Analysis of Petroleum Waxes by Gas Chromatography ("GC") or an equivalent gas chromatography method. From

these GC methods one of ordinary skill in the art is able to determine the weight percentages by standard integration techniques. A 95% carbon number spread between X and Y means that 95% of the carbon molecules (by weight) have a carbon number between the number X and the number Y.

In another embodiment, the present invention comprises a product that exhibits low shrinkage, low oil bleed, good color and texture and superior fragrance retention comprising about 75-95 wt %, preferably about 80-92.5 wt %, more preferably about 85-90 wt % of a midmelting point same refined wax produced by the ExxonMobil Raffinate Hydroconversion Process ("RHCTM") with the remainder being a high melting point fully refined wax.

#### DETAILED DESCRIPTION OF INVENTION

Traditionally candles have been made of petroleum derived Fully Refined Waxes (FRW) of different melting points. FRW are classified by their melting points. Those which melt at less than 128° F. (53° C.) are classified as Low Melting Point Fully Refined Waxes (LM FRW). Those which melt at between 128 to 145° F. (53-63° C.) are classified as Mid Melting Point Fully Refined Waxes (MM FRW). Those which melt at greater than 145° F. (63° C.) are classified as High Melting Point Fully Refined Waxes (HM FRW).

FIG. 1 shows a wax GC plot of the iso-paraffin content for a typical low-melting point FRW (MP 126° F.) used in container candle applications. This wax, which can be found commercially as ParVan™ 1270, has approximately 20% iso-paraffins with an average carbon number of about 28. This wax is translucent gray in color and exhibits approximately 15% shrinkage. This wax also has limited oil hold capacity, and sometimes requires candle formulation adjustments in order to hold higher levels of fragrance.

FIG. 2 shows a wax GC plot of the iso-paraffin content for a typical high-melting point FRW (MP 156° F.). This wax, commercially known as ParVan™ 1580, has approximately 50% iso-paraffins with an average carbon number of about 36. This wax is cloudy, gray white in color and exhibits approximately 6-8% shrinkage. Because of the inherent high MP and a typically higher market price, this wax is not commonly used for candles.

Another type of wax, mid-melt point RHCTM waxes have not been considered acceptable for use in candles due to their high oil content (1%-4%) and resulting problems of oil bleed and fragrance retention.

In the RHCTM process, which is detailed in U.S. Pat. No. 5,976,353 and U.S. Pat. No. 5,935,417 and are hereby incorporated by reference, lube raffinate is passed over a metal sulfide hydropyrolysis catalyst at relatively high temperature and pressure. Essentially all of the nitrogen and sulfur components of the feed stream are removed and a high percentage of the aromatic ring components are saturated to cyclo-paraffins. A limited amount of C—C bond cleavage (hydrocracking) also occurs in the RHCTM process. Collectively these changes in the raffinate feed stream provide lube basestock product with higher viscosity index and low aromatics levels, i.e., Group II basestocks.

Mid melt waxes separated from the RHCTM process has approximately 43%-57% iso-paraffins with an average carbon number of about 30-34. This wax is opaque-creamy white in color and exhibits exceedingly low shrinkage characteristics. Unfortunately, with its high oil content, the RHCTM wax was not useful for candles because it tended to demonstrate high oil bleed even before fragrance addition.

#### EXAMPLE 1

Hoping to take advantage of the low shrinkage and opaque white color characteristics of the MM RHCTM wax, while maintaining the low oil bleed and fragrance hold characteristics of the FRW, the inventors experimented with blends of the commercially available LM FRW 126, HM FRW 156 and MM RHCTM 135. The blends were selected to maintain a commercially viable final melting point and cost. Initial attempts to blend only a LM FRW wax and the MM RHCTM proved unsuccessful in controlling the oil bleed of the final blend. The inventors added a minor amount of a HM FRW 156 to the blends in an attempt to control the oil bleed by providing higher carbon number isoparaffins, similar to the effect expected from the addition of microwax but without the associated expense.

The wax blends were evaluated for shrinkage, oil bleed and color. All samples in all of the examples were prepared in identical glass jars. The jars were of a "stovepipe" configuration as shown in FIG. 3. Shrinkage was determined by filling the jars with the liquid wax blend to the fill line, which was located at the lower elbow of the jar, approximately 2 inches (5 cm) above the base. The molten wax was allowed to solidify at ambient temperature. Measurements were made by using an apparatus that aligned a metal measuring rod perpendicularly over the top of the jar. The measuring rod was lowered to determine how far below the fill line the lowest point of the top surface of the candle had fallen during solidification. Shrinkage measurements were reported in units of  $\frac{1}{16}$ th of an inch (1.59 mm).

The shape of the indentation is also reported. Conical means that the slope from the edge of the jar to the center was relatively constant. Concave means that the edge of the indentation was curved akin to a parabola. A sink hole means that part of the central portion of the indentation fell further and faster than the normal curvature, akin to a pothole or sinkhole. A center hump indicated that the indentation rose at the center. Oil bleed and color were determined by visual inspection. Surface oil means that small, typically pin-head sized, evenly spaced oil droplets were observed. Puddling means that larger, irregularly spaced drops typically greater than  $\frac{1}{4}$ " in diameter were observed.

Table 1 presents the results for various experimental blends. The blends shown in Table 1 were developed to meet a 130° F. MP typically used in container candles. As Table 1 demonstrates, no mixture of the three components performed adequately because there was significant shrinkage or oil bleed. For comparison, the shrinkage, oil bleed and appearance were determined for unblended FRW with melting points of 127° F. (52.7° C.) and 158° F. (70° C.) and an unblended MM HRC™ wax with a melting point of 135° F. (57.2° C.). These baseline characteristics are reported in Table 2.

#### EXAMPLE 2

60 A component study of the MM HRC™ 135, the LM FRW 126 and the HW FRW 156 using the same tests as used in the first example was conducted. Table 3 demonstrates the result that low shrinkage, low oil bleed and good color characteristics were found in a combination of the HM FRW 156 and the MM RHCTM 135 (blends 1168 and 1170). This result was surprising because, as noted above, one of ordinary skill in the art would not consider the use of HM FRW in a candle.

TABLE 1

| blend:                                     | 1147                                  | 1148                        | 1149                  | 1150                        | 1151                           | 1152                                | 1153                                                   |
|--------------------------------------------|---------------------------------------|-----------------------------|-----------------------|-----------------------------|--------------------------------|-------------------------------------|--------------------------------------------------------|
| MM RHC™ (wt %)<br>(MP 135° F.)             | 25                                    | 35                          | 30                    | 30                          | 40                             | 50                                  | 60                                                     |
| LM FRW (wt %)<br>(MP 126° F.)              | 72.5                                  | 60                          | 60                    | 65                          | 50                             | 40                                  | 30                                                     |
| HM FRW (wt %)<br>(MP 157° F.)              | 2.5                                   | 5.0                         | 10                    | 5.0                         | 10                             | 10                                  | 10                                                     |
|                                            |                                       |                             |                       |                             |                                |                                     |                                                        |
| Total                                      | 100                                   | 100                         | 100                   | 100                         | 100                            | 100                                 | 100                                                    |
| Melting Point of<br>Blend ° F. (° C.)      | 126 (52.2)                            | 127 (52.7)                  | 128 (53.3)            | 127 (52.7)                  | 129 (53.9)                     | 130 (54.4)                          | 131 (55.0)                                             |
| Shrinkage in $\frac{1}{16}$ "<br>(1.59 mm) | 5                                     | 5                           | 10                    | 5                           | 7                              | 9                                   | 10                                                     |
| Top Surface Shape                          | Concave<br>Center Hump<br>Surface Oil | Concave                     | Conical               | Concave                     | Concave                        | Concave<br>Sink Hole<br>Surface Oil | Concave<br>Sink Hole<br>Surface Oil<br>and<br>Puddling |
| Oil Bleed                                  | Surface Oil                           | Surface Oil<br>and Puddling | None                  | Surface Oil<br>and Puddling | Surface Oil<br>and<br>Puddling | Surface Oil<br>and<br>Puddling      | Surface Oil<br>and<br>Puddling                         |
| Color and Texture                          | Cloudy Gray<br>Smooth                 | Cloudy Gray<br>Smooth       | Cloudy Gray<br>Smooth | Cloudy Gray<br>Smooth       | Cloudy<br>Gray-White<br>Smooth | Cloudy<br>Gray-White<br>Smooth      | Cloudy<br>Gray-White<br>Smooth                         |

EXAMPLE 3

TABLE 2

| blend:                                        | 02-9201                       | 02-78026                      | 03-3022                          |
|-----------------------------------------------|-------------------------------|-------------------------------|----------------------------------|
| ProWax™ 320 (wt %)<br>(MM RHC) (M.P. 135° F.) | —                             | —                             | 100                              |
| PV 1270 (wt %)<br>(LM FRW) (M.P. 127° F.)     | 100                           | —                             | —                                |
| PV 1580 (wt %)<br>(HM FRW) (M.P. 158° F.)     | —                             | 100                           | —                                |
| Shrinkage in $\frac{1}{16}$ "<br>(1.59 mm)    | 10                            | 5                             | 2                                |
| Top Surface Shape                             | Conical                       | Concave                       | Slightly<br>Concave              |
| Oil Bleed                                     | None                          | None                          | Surface Oil<br>and Puddling      |
| Color and Texture                             | Translucent<br>Gray<br>Smooth | Translucent<br>Gray<br>Smooth | Opaque White<br>Creamy<br>Smooth |

25 The inventors were surprised by the results of the component study showing that a HM FRW and the MM HRC™ provided the inventive results of low shrinkage and no oil bleed without the addition of a LM FRW. However, striving for commercial acceptance, the inventors desired to find the lowest possible melting point FRW that could be used and still provide the present invention. However, as Table 4 demonstrates, the effect of low shrinkage, good color and no bleed retention is surprisingly only achieved with a mixture of the MM HRC™ and a HM FRW with a MP of greater than about 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9

TABLE 4

| Sample | Compositional Information (wt %) |           |           |                   |           |           |           | Shrink Depth<br>(in $\frac{1}{16}$ ') | Color/<br>Texture                                                                 |
|--------|----------------------------------|-----------|-----------|-------------------|-----------|-----------|-----------|---------------------------------------|-----------------------------------------------------------------------------------|
|        | MM<br>RHC                        | LM<br>FRW | LM<br>FRW | LM<br>FRW<br>M.P. | MM<br>FRW | MM<br>FRW | HM<br>FRW |                                       |                                                                                   |
| 1245   | 90                               | 10        |           |                   |           |           |           | 12                                    | Concave,<br>sink hole<br>Surface<br>oil and<br>puddling<br>cloudy gray,<br>smooth |
| 1251   | 90                               |           | 10        |                   |           |           |           | 12                                    | Concave,<br>sink hole<br>Surface<br>oil and<br>puddling<br>cloudy gray,<br>smooth |
| 1248   | 90                               |           | 10        |                   |           |           |           | 10                                    | Concave,<br>sink hole<br>Surface<br>oil and<br>puddling<br>cloudy gray,<br>smooth |
| 1254   | 90                               |           |           | 10                |           |           |           | 9                                     | Concave,<br>sink hole<br>Surface<br>oil and<br>puddling<br>cloudy gray,<br>smooth |
| 1194   | 90                               |           |           |                   | 10        |           |           | 5                                     | Concave,<br>sink hole<br>Surface<br>oil and<br>puddling<br>cloudy gray,<br>smooth |
| 1220   | 90                               |           |           |                   |           | 10        |           | 5                                     | Concave<br>None<br>opaque<br>white,<br>creamy<br>smooth                           |

TABLE 5

| Claimed Ranges for              | MM RHC | HM FRW |
|---------------------------------|--------|--------|
| Avg. Carbon # (Total Paraffins) | 29-33  | 36-40  |
| Avg. Carbon # (iso-Paraffin)    | 30-34  | 38-42  |
| % n-Paraffin                    | 43-57  | 43-57  |
| 95% Carbon # Spread             | 12-16  | 19-25  |
| % C24-                          | <10    | <5     |
| % C34+                          | <30    | >60    |
| % C38+                          | <10    | >40    |

Upon further analysis, the inventors realized that this surprising result would be produced by producing a wax blend of about 75-95 wt %, preferably about 80-92.5 wt %, more preferably about 85-90 wt % of a wax with parameters similar to those in Column A of Table 5, the remainder being a wax with parameters similar to those in Column B of Table 5.

#### EXAMPLE 4

With further experimentation, the inventors realized that an increase in the wt % iso-paraffin for the carbon number from about 36 to about 60, preferably from about 36 to 57, more preferably from about 37 to 55 and even more preferably from about 37 to 50, without the attendant increases (greater than about 1 wt %) in the same at carbon number greater than 60, preferably greater than 57, more preferably greater than 55, even more preferably greater than 50 produced the remarkable results of low shrinkage, little to no oil bleed, excellent color and expected excellent fragrance retention. Due to this unexpected result of Example 3, the inventors conducted additional gas chromatography experiments. FIG. 4 shows the weight % of isoparaffins in each wax at each carbon number for four waxes, a LM FRW 126, a MM RHC™ 135, a HM FRW 156 and for a 90:10 blend of the MM RHC™ 135 and the HM FRW 156.

The inventors noted that blend LS 1360 was very similar to MM HRC™ with one notable difference: the increase in the weight % iso-paraffins for carbon number from about 36 to about 60. The inventors compared this to a GC of microwax as

shown in FIG. 6, as microwax was often used to control oil bleed but leads to shrinkage. FIG. 6 shows that microwax starts to show isoparaffins about carbon number 34 which increase steadily to carbon number 50 with approximately 40% of the iso-paraffins having a carbon number of 50 or greater. This experiment indicates that the advantages of less shrinkage and no oil bleed can be achieved when one does not follow the industry tradition of using microwax, which would increase the weight percentage of the isoparaffins with a carbon number of greater than 50 and in the final blend by more than about 0.1 wt % at a given carbon number.

What is claimed is:

1. A wax blend comprising:
  - (a) about 75-95 wt % of a first wax wherein said first wax has:
    - i) a melting point of between about 128° F. to about 145° F.;
    - ii) an oil content of between about 1 wt % to about 10 wt %;
    - iii) a total paraffins average carbon number of between about 29-33;
    - iv) an iso-paraffin average carbon number of between about 30-34;
    - v) about 43-57 wt % n-paraffins;
    - vi) a 95% carbon number spread of 12-16;
    - vii) the weight percent of said first wax's molecules having a carbon number of C24 or less being less than about 10%;
    - viii) the weight percent of said first wax's molecules having a carbon number of C34 or greater being less than about 30%;
    - ix) the weight percent of said first wax's molecules having a carbon number of C38 or greater being less than about 10%; and
  - (b) the remainder being a second wax wherein said second wax has:
    - i) a melting point greater than about 152° F.;
    - ii) an oil content of less than about 1 wt %;
    - iii) a total paraffins average carbon number of between about 36-40

**11**

- iv) an iso-paraffin average carbon number of between about 38-42;
  - v) about 43-57 wt % n-paraffins;
  - vi) a 95% carbon number spread of 19-26;
  - vii) the weight percent of said second wax's molecules having a carbon number of C24 or less being less than about 5%;
  - viii) the weight percent of said second wax's molecules having a carbon number of C34 or greater being greater than about 60%; and
  - ix) the weight percent of said second wax's molecules having a carbon number of C38 or greater being greater than about 40%.
2. The wax blend of claim 1 wherein said melting point of said first wax is between about 129° F. and about 140° F. 15
3. The wax blend of claim 1 wherein said melting point of said second wax is greater than about 156° F.

**12**

- 4. The wax blend of claim 1 wherein the oil content of the first wax is between about 1 wt % and about 7 wt %.
- 5. The wax blend of claim 1 wherein the oil content of the second wax is less than about 0.8%.
- 6. The wax blend of claim 1 wherein said first wax comprises about 80 to 92.5 wt % of the total blend.
- 7. The wax blend of claim 1 wherein said first wax comprises about 85 to 90 wt % of the total blend.
- 8. The wax blend of claim 1 wherein said melting point of said first wax is between about 131° F. and 139° F.
- 9. The wax blend of claim 1 wherein the oil content of the first wax is between about 1 wt % and about 5 wt %.
- 10. The wax blend of claim 1 wherein the oil content of the second wax is less than about 0.5 wt %.
- 11. The wax blend of claims 1, 2, 3, 4, 5, 6, 7, 8, 9 or 10 wherein said first wax is derived from the ExxonMobil Raffinate Hydroconversion Process™.

\* \* \* \* \*